

## UNITED STATES PATENT OFFICE

2,455,954

## PROCESS FOR PRODUCING WHITE CAST IRON CASTINGS

Oliver Smalley, Larchmont, N. Y., assignor to  
Meehanite Metal CorporationNo Drawing. Application September 22, 1945,  
Serial No. 618,059

3 Claims. (CL. 75—130)

1

My invention relates to the process of the manufacture of cast iron, with or without alloying agents, under such control as to produce white iron castings that combine both hardness and toughness.

By white iron, I mean a cast iron—alloy or otherwise—in which the bulk or all of the carbon is present in the form of iron carbide and which presents a white fracture.

White iron castings being rarely machined and selling at low competitive prices, have not advanced technologically and industrially during the past decade as have gray cast iron castings. Generally white iron castings are the most unpredictable products of the foundry industry and the idea has existed that an iron giving a white fracture is suitable for any type of hard wear service, and may be defined as white iron. In other words, the idea has prevailed, and still prevails in certain quarters, that if an iron fractures white, then the metal is a serviceable material for abrasion resisting conditions and perhaps for heat resisting purposes because it is substantially free from flake graphite or that it can be malleabilized by prolonged annealing above the critical point.

White iron is however, not a specific material but rather a generic term. An iron that breaks with a white fracture may be extremely brittle or it may be reasonably tough. It may present superior or inferior resistance to abrasion. Under heat influence, it may stand up reasonably well or it may fail prematurely. It may malleabilize in a standard annealing time and give good combined strength and ductility, or its response to a malleabilizing treatment may be quite unsatisfactory and inferior properties frequently result.

White iron is commonly made by adjusting the carbon and silicon to suitable ratio, or it may be produced by the simple expedient of adding carbide-forming elements, for example, chromium, tellurium, uranium, vanadium, and sulphur, all of which influence differently the ultimate serviceable value of the product.

Whichever method is used, the end product is usually an indeterminate material of uncertain properties. If it is to be used for abrasion resisting purposes its B. H. N. value may vary from 350 to 578. Its strength properties may differ as much as 100% or more, and the casting difficulties encountered often result in rejection of the casting because of the problems of overcoming shrinkage defects and weakness dependent on uncontrolled development of grain structure.

2

The basis of this invention is a process which is so controlled as to produce a casting to a predetermined degree of whiteness of known physical characteristics that has uniform liquid shrinkage for casting purposes and is free from columnar grain weakness and in which the degree of hardness and strength properties bear a direct relation to the sectional dimension and shape of the finished casting.

10. An object of my invention is to produce a white iron to a predetermined and controlled degree of whiteness and of known physical characteristics.

Another object of my invention is to produce a white iron that is free from crystal weakness and inherent brittleness.

Another object of my invention is to produce a white iron whose structure is mainly equiaxed as distinct from the uncertain unbalanced columnar growth common to ordinary white iron.

20. A further object of my invention is to produce a white iron to a predetermined abrasion resisting characteristic which is substantially constant regardless of the sectional dimensions of the finished casting.

Another object of my invention is to produce a white iron casting free from shrink voids and mechanical weakness.

Another object of my invention is to produce a white iron casting whose heat resisting properties are under control and of assured service life value.

30. Another object of my invention is to produce a white iron casting of known physical structure which can be malleabilized by annealing at a given temperature and time to assure dependable reaction to malleabilizing treatment.

Another object of my invention is a two-step process for the manufacture of white iron castings, the first step comprising selecting a mixture of raw materials which when melted will have a structural constitution bearing a direct relationship to the thickness of the sections to be cast, and the second step comprising altering or modifying the massive cementite to produce a final structure that possesses the desired improved degree of toughness.

Another object of my invention is to give positive control over the physical properties in a white iron casting, comprising the control and measurement of constitutional carbide values and processed carbide values, and regulating through said control the relation of the constitutional and process carbide values to each other and to the thickness of the casting to be made.

Other objects and a fuller understanding of my invention may be had by referring to the following description and claims:

The process of my invention comprises two steps. The first step may be characterized as determining the constitutional carbide value of the melt and the second step may be characterized as determining the processed carbide value. Both steps are related to the thickness of the casting to be made. The first step of the process comprises selecting a mixture of raw materials which when melted will yield a constitutional carbide value which will bear a direct relationship to the thickness of the casting to be made. The second step comprises treating the molten iron to a predetermined carbide value but maintaining the iron in condition to produce a white casting.

In my invention, the structural components of the iron, one with another, are established according to the thickness and design of the casting to be made. One method of establishing the constitution and the processed carbide values of the metal may be explained as follows: I preferably determine the constitutional carbide value and the processed carbide value by a wedge test or its equivalent. The constitutional carbide value of the iron measured by the wedge test may be, for example  $(4\frac{1}{2}\%)$ . The wedge test comprises the pouring of a specimen of a predetermined length and of wedge form in cross-section with an acute angle of approximately 20 to 30 degrees. The wedges may be of several sizes, namely, one-half inch base with approximately  $28.5^\circ$  acute angle, three-fourths inch base with approximately  $26.75^\circ$  acute angle, one inch base with approximately  $25^\circ$  acute angle, and two inch base with approximately  $23.5^\circ$  acute angle. Wedges with larger bases have proportionately smaller acute angles. After the wedge test specimen is poured from the melt and cooled, it is broken in two so that the constitutional carbide value may be observed. Upon observation, one can discern that the acute angle portion has a white appearance while the remaining base portion has a gray appearance. In the white portion, the carbon is substantially in combined form, and in the gray portion a large percentage of its carbon is in the form of graphite. The width across the face of the wedge at the line of demarcation between the white and the gray portion is a measure of the constitutional carbide value of the iron. Thus, in the example of the iron above, the wedge measured  $(4\frac{1}{2}\%)$  inch across the face thereof at the line of demarcation. The wedge sizes are so proportioned that the distance across any one of the wedges at the line of demarcation is substantially the same for the metal having the same carbide value. In other words, the constitution of the iron as measured by the wedge test is the same regardless of the particular size of standardized wedge used to make the test. The distance across the face of the wedge at the line of the demarcation between the white and the gray iron is sometimes referred to as the constitutional carbide wedge value, or more preferably as constitutional wedge value. The line of demarcation between the white and the gray iron as measured by the wedge test is also a measurement or indication of the sensitivity to chilling from the molten condition to room temperature.

In order that a constitutional carbide value of  $(4\frac{1}{2}\%)$  may be observed, the molten metal would be poured into a two-inch, or larger, standard wedge, in which event the demarcation between the white

and the gray iron would be one and one-half inches long, thus  $(4\frac{1}{2}\%)$ .

By processing the molten metal, the wedge specimen will have a new line of demarcation, which may be, for example,  $(3\frac{1}{2}\%)$ . The processing of the molten metal may be done by any well-known method and may comprise the mixing of nucleating agents with the molten metal as it flows from the cupola or in the ladle but prior to the time at which the metal is solidified in the molds. The processed metal when poured into a casting of wedge form shows a new or different line of demarcation between the white iron and the gray iron, in that the line of demarcation is shifted toward the knife edge of the wedge. Thus, when an iron is said to be processed to a  $(3\frac{1}{2}\%)$  wedge, it means that the distance across the face of the wedge at the line of demarcation is  $(3\frac{1}{2}\%)$  of an inch, namely one and one-eighth inches, and is, in simple terms, referred to as a  $(3\frac{1}{2}\%)$  wedge. Technically, the distance across the face of the wedge at the new line of demarcation is referred to as processed carbide wedge value or processed wedge value, as distinguished from constitutional wedge value. The distance at the new line of demarcation or the processed wedge value is a measurement or indication of the sensitivity to chilling from the molten condition and bears a direct ratio to the thickness of the casting to be made.

When the line of demarcation between the gray and the white iron on a wedge specimen is substantially  $(2\frac{1}{2}\%)$ , and when this iron is poured into a one inch section of generally rectangular shape, it will be substantially or nearly all white, and this whiteness may be designated as whiteness of 1-times white. In other words, in order that a casting of one inch thickness  $(2\frac{1}{2}\%)$  and of generally rectangular shape may fracture just all white; that is, 1-times white, the equivalent value for the wedge is substantially  $(2\frac{1}{2}\%)$ . The wedge value is substantially  $1\frac{1}{2}$  times the thickness of the section to be cast. Thus, for a casting to fracture 1-times white, it is found that the wedge value for the iron is substantially  $1\frac{1}{2}$  times the thickness of the section of the casting to be made. Further, when the line of demarcation on a wedge specimen is substantially  $(7\frac{1}{2}\%)$ , and when this iron is poured into a one-inch section of generally rectangular shape, the one-inch section will fracture all white, and the whiteness may be designated as whiteness of 2-times white. If the metal having a wedge value of  $(7\frac{1}{2}\%)$  is poured into a 2-inch section of generally rectangular shape, the 2-inch section will fracture all white and the whiteness may be designated as whiteness of 1-times white. Also, when the line of demarcation on a wedge specimen is substantially  $(10\frac{1}{2}\%)$  and when this iron is poured into a section of one inch of generally rectangular shape, the section will, of course, fracture all white, and the whiteness may be designated as whiteness of 3-times white. If the metal having a wedge value of  $(10\frac{1}{2}\%)$  is poured into a 3-inch section of generally rectangular shape, the 3-inch section will fracture all white and the whiteness may be designated as whiteness of 1-times white. This nomenclature may be extended to include the whiteness of the fourth, fifth, or higher order, or fractions thereof.

The constitutional carbide value and the processed carbide value bear a relationship to each other and to the thickness of the casting to be made. Thus, castings of different sections are made with different constitutional and processed values. The values for making finished castings

having substantially one-inch sections will be illustrated first. Sections of other dimensions will bear a direct ratio to the values for a one-inch section. For castings having substantially one-inch sections, my invention is practiced by first preparing molten metal which, when tested, produces a constitutional carbide wedge value embraced within a range having a minimum value of substantially  $(4\frac{4}{32})$  and a maximum value as hereinafter defined. A wedge value of  $(4\frac{4}{32})$  is substantially equivalent to  $1\frac{1}{4}$  times white in a casting of substantially one inch thick and of generally rectangular shape. Next, I process the molten metal which, when tested, produces a processed carbide value embraced in a range having a minimum value of substantially  $(3\frac{3}{32})$  and a maximum value of  $(9\frac{9}{32})$ . A wedge value of  $(3\frac{3}{32})$  is equivalent to 1-times white in a casting of substantially one inch thick and of generally rectangular shape and a wedge value of  $(9\frac{9}{32})$  is substantially equivalent to  $2\frac{1}{2}$ -times white. The maximum value of the constitutional carbide value may not be greater than three times the maximum process carbide value. The maximum value for the constitutional carbide would be not greater than  $(27\frac{7}{32})$ . A wedge value of  $(27\frac{7}{32})$  is substantially equivalent to  $7\frac{1}{2}$ -times white in a casting of one inch thick and of generally rectangular shape.

Corresponding proportionate wedge values would obtain for sections of different thickness. Thus, for castings of substantially 2 inches thick, the wedge values given above would be doubled, in which case, for example, the minimum constitutional wedge value for a 2-inch section would be  $(8\frac{8}{32})$ . A wedge value of  $(8\frac{8}{32})$  is substantially equivalent to  $1\frac{1}{4}$ -times white in a casting of substantially 2 inches thick and of generally rectangular shape. Other wedge values with respect to the thickness of castings will bear the same ratio as those set forth above for a 1-inch section.

From the above wedge values, it is noted that the minimum constitutional wedge value is substantially  $1\frac{1}{2}$  times the section of a finished casting. The minimum processed wedge value is substantially  $1\frac{1}{8}$  times the section of the finished casting and the maximum processed carbide wedge value is substantially  $2\frac{1}{4}$  times the average section of the casting to be made. The maximum constitutional wedge value is less than 3 times the maximum value of the processed wedge value.

The wedge values as given above may be translated in terms of the degree of whiteness of a casting of generally rectangular section, in which case the constitutional carbide value is embraced within a range having a minimum value of  $1\frac{1}{4}$ -times white and a maximum value as hereinafter specified. The processed carbide values would be embraced within a range having a minimum value of 1-times white to  $2\frac{1}{2}$ -times white. The maximum value of the constitutional carbide value would be not greater than 3 times the maximum processed carbide value.

Any white iron casting that is made having a constitutional carbide value and a processed carbide value falling within the limits of the above defined ranges, will have good wear resisting qualities and yet be tough. White iron castings made by values which lie close to the minimum values of the range of values will have somewhat different properties than white iron castings made by values lying close to the maximum values of the ranges given above. A range which may

represent mean values for making white iron castings may be as follows:

| Thickness of Section                          | $\frac{1}{4}$ inch | 1 inch          | $1\frac{1}{2}$ inch |
|-----------------------------------------------|--------------------|-----------------|---------------------|
| 5 Minimum Constitutional Carbide Wedge Value  | $2\frac{1}{32}$    | $4\frac{5}{32}$ | $8\frac{9}{32}$     |
| 10 Maximum Constitutional Carbide Wedge Value | $5\frac{9}{32}$    | $9\frac{9}{32}$ | $19\frac{7}{32}$    |
| 10 Minimum Processed Carbide Wedge Value      | $2\frac{9}{32}$    | $4\frac{9}{32}$ | $7\frac{2}{32}$     |
| 10 Maximum Processed Carbide Wedge Value      | $4\frac{9}{32}$    | $8\frac{9}{32}$ | $18\frac{9}{32}$    |

White iron castings controlled by values lying in the mean range given above will have a high resistance to wear and yet be tough and strong so that they will have resistance to fracture under heavy physical impacts.

In practicing my invention, the foundry operator first melts a charge or otherwise prepares a mixture of molten materials which, when tested, gives a constitutional value lying within the range of the values hereinabove specified with relation to the thickness of the castings to be made. Next, the operator processes the molten material which, when tested, gives a processed carbide value lying within the range of the values hereinabove specified with respect to the thickness of the castings to be made. Having satisfied that the molten metal meets the above requirements, the operator may now pour the processed metal in the mold for making the finished white iron castings.

The foundry operator, in the practice of my invention, is able to produce white iron castings having a controlled degree of whiteness whereby castings made under my process have high abrasion and heat resisting characteristics which will assure long service life value. The castings will also have the proper characteristics, whereby they can be malleablized by annealing at any given temperature and time and assure dependable reaction to malleablizing treatment.

Although I have described my invention in its preferred form with a certain degree of particularity, it is understood that the present disclosure of the preferred form has been made only by way of example and that numerous changes in the details of the process, modification in the steps undertaken, variations in the materials used, and different values of wedges establishing carbide balance, may be resorted to without departing from the spirit and the scope of the invention as hereinafter claimed.

I claim as my invention:

1. A process to give positive control of the physical properties in a white iron casting which comprises providing molten cast iron which when cast in a wedge shaped test piece and then broken in two, exhibits upon the broken faces both gray and white iron with a line of demarcation therebetween of such a length as to be embraced within a range having a minimum value of more than  $1\frac{1}{2}$  times the average section to be made and a maximum value as hereinafter specified, processing the molten material which when cast in a wedge shaped test piece and then broken in two, exhibits upon the broken faces a larger amount of gray iron and a smaller amount of white iron with a new and shorter line of demarcation than that exhibited on the first mentioned test piece, said new line of demarcation being of such length as to be embraced within a range having a minimum value of more than  $1\frac{1}{8}$  times the average section of the casting to be made and a maximum value of less than  $2\frac{3}{4}$  times the average section of the casting to be made, said

maximum value of the constitutional carbide value being not greater than 3 times the maximum processed carbide value hereinabove specified.

2. A process to give positive control of the physical properties in a white iron casting which comprises providing molten cast iron which produces a constitutional carbide value embraced within a range having a minimum value of 1½-times white and a maximum value as hereinafter defined, and processing the molten cast iron to produce a processed carbide value embraced in a range having a minimum value of 1-times white and a maximum value of 2½-times white, said maximum value of the constitutional carbide value being not greater than three times the maximum process carbide value hereinabove specified.

3. A process to give positive control of the physical properties in a white iron casting which comprises providing molten cast iron which produces a constitutional carbide wedge value embraced in a range having a minimum value of at least substantially  $2\frac{1}{2}$  for castings  $\frac{1}{2}$ -inch thick,  $4\frac{1}{2}$  for castings substantially 1-inch thick and  $8\frac{1}{2}$  for castings substantially 2-inches thick and having a maximum value of at least substantially

$5\frac{1}{2}$  for castings substantially  $\frac{1}{2}$ -inch thick,  $9\frac{1}{2}$  for castings substantially 1-inch thick, and  $19\frac{1}{2}$  for castings substantially 2-inches thick, and processing the molten material to give a processed carbide wedge value embraced within a range having a minimum value of at least substantially  $20\frac{1}{2}$  for castings substantially  $\frac{1}{2}$ -inch thick,  $40\frac{1}{2}$  for castings substantially 1-inch thick,  $80\frac{1}{2}$  for castings substantially 2-inches thick and  $160\frac{1}{2}$  for castings substantially 2-inches thick.

OLIVER SMALLEY.

#### REFERENCES CITED

The following references are of record in the file of this patent:

#### UNITED STATES PATENTS

| Number    | Name           | Date          |
|-----------|----------------|---------------|
| 2,371,654 | Smalley et al. | Mar. 20, 1945 |

#### FOREIGN PATENTS

| Number  | Country   | Date          |
|---------|-----------|---------------|
| 105,619 | Australia | Oct. 25, 1938 |